

# UNITED STATES PATENT OFFICE.

RALPH E. MYERS AND ROY D. HALL, OF EAST ORANGE, NEW JERSEY, ASSIGNEES  
TO WESTINGHOUSE LAMP COMPANY, A CORPORATION OF PENNSYLVANIA.

## FILAMENT FOR INCANDESCENT ELECTRIC LAMPS.

1,363,162.

Specification of Letters Patent. Patented Dec. 21, 1920.

No Drawing.

Application filed May 14, 1915. Serial No. 28,163.

To all whom it may concern:

Be it known that we, RALPH E. MYERS, a citizen of the United States, and a resident of East Orange, in the county of Essex and State of New Jersey, and ROY D. HALL, a citizen of the United States, and a resident of East Orange, in the county of Essex and State of New Jersey, have invented a new and useful Improvement in Filaments for Incandescent Electric Lamps, of which the following is a specification.

Our invention relates to the manufacture of filamentary material, and it has special reference to such filaments as constitute incandescent bodies for electric lamps.

The object of our invention is to provide filaments of the above-indicated character which shall possess good electrical properties and which shall likewise be durable and resistant to mechanical shocks and to structural changes resulting from the passage of electric current through the filaments.

More particularly, the object of our invention is to provide metallic filaments, composed largely or mainly of metals of the tungsten type, which shall be highly resistant to the structural alterations known as "offsetting" or "faulting" that tend to develop in this class of filaments during their use.

Certain materials which are suitable for use as filaments for incandescent electric lamps have considerable mechanical strength when first formed into filaments but become exceedingly fragile after they have been traversed by electric currents. This phenomenon is a characteristic of tungsten filaments, whether such filaments are prepared by squirting or drawing processes, and it is found that pure tungsten filaments which have considerable initial strength and which, in the case of drawn tungsten wire, may even have a tensile strength many times exceeding that of steel, become brittle after being traversed by current for a few hundred hours. The filaments are therefore easily broken and, upon microscopic examination, they are found to have undergone marked structural alterations. The outline of such a filament shows lateral displacement of sections of the filament relative to one another, and this displaced condition, which is known in the art as "offsetting" or "faulting," appears to be caused by the development and

growth of crystals within the body of the filament. Such crystals seem to increase in size in much the same manner as crystals formed in liquid solutions, and, if the crystals become large enough to extend almost or entirely across the filament, adjacent crystals tend to slip along their cleavage planes, thereby giving the filament the offset of faulted appearance above referred to. It therefore appears that internal crystallization produces offsetting and that offsetting imparts brittleness to the filaments.

The phenomenon described above becomes a particularly serious problem in the manufacture of slender metallic filaments which are used in the smaller types of incandescent lamps such as 25-watt, 40-watt and similar lamps.

An efficient method of resisting offsetting in lamp filaments was proposed by Dr. Anton Lederer and described in United States Patent, #1,180,264 and assigned to the Westinghouse Lamp Company.

According to Dr. Lederer's method, and according to the technical practice heretofore prevailing, the preferred addition materials are the oxides of the rare earth metals, particularly thorium oxid.

We have discovered that the offsetting of lamp filaments may be effectively prevented by the addition of small amounts of other refractory substances which neither volatilize nor decompose under the conditions existing in glowing incandescent filaments. The substances which we have discovered to be particularly suitable for this purpose are the oxides of the alkali metals, the alkaline earths, and also certain oxides belonging to neither of these classes, such as beryllium oxid, aluminum oxid and titanium oxid,  $TiO_2$ . For the present purpose, we include magnesium oxid among the alkaline earths, as well as calcium oxid, barium oxid and strontium oxid. Of the alkali metal oxides, we have found lithium oxid to be particularly effective, and of the alkaline earth oxides, calcium oxid and magnesium oxid are especially suited to our purpose.

We have found also that excellent results may be obtained by the use of mixtures of two or more of the substances enumerated above, or mixtures of one or more of these substances with one or more oxides of rare earth metals, including thorium oxid. Very

satisfactory results have been obtained by using calcium oxide and magnesium oxide as the additive materials. Such mixtures give superior results in some cases, although the 5 reason why such improved results are obtained with mixtures is not clear.

Our invention is of special importance in the manufacture of tungsten filaments, but it may also be applied to filaments composed 10 of other metals, such as molybdenum, tantalum and the like.

Very small amounts of offset-resisting materials are sufficient to greatly retard the development of offsetting. A few hundredths of one per cent. are sometimes sufficient, and it is usually unnecessary to add to the filaments more than 5% of their weight of the offset-resisting additions in order to obtain the maximum offset-resist- 20 ing effect.

The addition of the offset-resisting materials may be made at any desired stage of the manufacture of the filaments, but in making drawn tungsten filaments, we ordi- 25 narily find it convenient to add the offset-resisting materials to the powdered oxid before it is reduced to metal. The precise steps

of the process of forming filaments by drawing, squirting or otherwise form no part of our present invention. It is also to be understood that other limitations are not to be imposed thereon except as indicated in the appended claims.

We claim as our invention:

1. A filament comprising drawn tungsten 35 wire that tends to offset when utilized as a conductor of electricity and also containing calcium oxide and magnesium oxide.

2. A filament comprising tungsten that tends to offset when utilized as a conductor 40 of electricity and also containing at least two of a group of substances including the alkali metal oxides, the alkaline earths, beryllium oxide, aluminum oxide, and titanium dioxide.

In testimony whereof we have hereunto subscribed our name this 30th day of April, 1915.

RALPH E. MYERS.  
ROY D. HALL.

Witnesses:

ALFRED H. EDGERLEY,  
FREDERICK A. BETTS.